

# United States Patent

[11] 3,615,324

[72] Inventors William D. Gordon  
Lynn;  
Robert S. Norman, Marblehead, both of  
Mass.  
[21] Appl. No. 741,935  
[22] Filed July 2, 1968  
[45] Patented Oct. 26, 1971  
[73] Assignee General Electric Company

3,031,522 4/1962 Clark et al. .... 174/102  
Primary Examiner—S. Leon Bashore  
Assistant Examiner—Saul R. Friedman  
Attorneys—Richard E. Hosley, Melvin M. Goldenberg, Frank  
L. Neuhauser and Oscar B. Waddell

[54] **PROCESS FOR FORMING HERMETIC SEAL FOR  
SHEATHED ELECTRICAL CONDUCTORS**  
5 Claims, 4 Drawing Figs.

[52] U.S. Cl. .... 65/36,  
65/59, 174/102  
[51] Int. Cl. .... C03c 27/02,  
C03c 17/00  
[50] Field of Search. .... 65/36, 59;  
174/102; 29/472.9, 474.4

[56] **References Cited**  
UNITED STATES PATENTS  
2,962,684 11/1960 Lien, Jr. .... 65/36 X

**ABSTRACT:** A process for forming a hermetic seal from a finely pulverized mixture of glass and 30-40 percent by weight of magnesium oxide. A finely pulverized mixture of a lead-potash-soda glass with 30-40 percent by weight of magnesium oxide is loaded into the area around the electrical conductors to be sealed. The powdered mixture is "pressed" to reduce porosity and compact the particles. Thereafter, the mixture is heated to a temperature which drives off moisture and purges air from the mixture. Thereafter, the temperature is elevated at a rate to induce crystallization in the material without causing stratification while raising the temperature to the working point of the glass in the seal mixture. Thereafter, the composition is cooled until it becomes rigid.



FIG. 1

PRIOR ART



FIG. 2

## MIXING OPERATION

FINELY PULVERIZED GLASS AND 30% TO 40%  
FINELY PULVERIZED  $MgO$  MIXED TO  
HOMOGENEOUS SEAL MIXTURE

## ASSEMBLY OPERATION

SEAL MIXTURE PLACED IN SHEATHED  
CONDUCTOR IN CONTACT WITH INSULANT

## COMPACTING OPERATION

SEAL MIXTURE PLACED UNDER PRESSURE TO  
REDUCE POROSITY AND PROVIDE INTIMATE  
CONTACT

## HEAT TREATMENT OPERATION

TEMPERATURE OF ASSEMBLY RAISED TO  
WORKING POINT OF GLASS IN SEAL  
MIXTURE AND THEN COOLED

FIG. 4



FIG. 3



INVENTORS

WILLIAM D. GORDON

ROBERT S. NORMAN

BY

Richard C. Horsley

ATTORNEY

## PROCESS FOR FORMING HERMETIC SEAL FOR SHEATHED ELECTRICAL CONDUCTORS

### BACKGROUND OF THE INVENTION

This invention relates to sheathed electrical conductors having a hermetic sealing structure and is particularly concerned with a method for making such conductors. This application is a division of application Ser. No. 618,168 filed Feb. 23, 1967 now Pat. No. 3,451,861, issued June 24, 1969.

The sheathed conductors of the type with which the present invention is concerned are those designed for high temperature applications in which one or more conductors are enclosed within a tubular metallic sheath and supported in spaced relation within the sheath by a layer of heat refractory, electrically insulating material. Specific embodiments of such sheathed conductors may take the form of thermocouple assemblies, spark plug connecting leads or the like.

Measurements of temperatures within high temperature power plants, such as aircraft gas turbines, are customarily made with temperature detectors employing thermocouples having conductors sheathed in a cylindrical metallic housing or barrel tightly packed with refractory insulating powder or a substantially solid ceramic core. Such thermocouples were necessarily of the most rugged construction to avoid rapid deterioration under extreme vibration and temperature conditions. However, for speed of response to rapid variations in the measured temperature, the thermocouple junction of the conductors in such temperature detectors usually extended beyond the end of the outer metallic housing through an opening in the end of that housing, and the insulating core would thus be exposed to fuel. When this occurred, the fuel penetrated the core and was drawn into the upper portions of the barrel where subsequent rapid heating could carbonize the fuel. Water vapor released by the combustion of the fuel also was drawn into the insulating material of the core in the same manner, and the result of this carbonization and the hydration was harmful because it could reduce the resistance between the conductors or between the sheath and the conductors. The principal reason behind this type of failure in thermocouple assemblies was found to lie in the necessity of exposing at least a portion of the insulant filling metallic sheath to the fuel and water vapor.

To provide a solution for this type of problem, a thermocouple assembly having a core of insulating material comprising glass and magnesium oxide was developed. Such an insulating material for sheathed electrical conductors is thoroughly described and the method for making such a sheathed conductor claimed in U.S. Pat. No. 3,031,522, issued Apr. 24, 1962, to Robert B. Clark et al. and assigned to the same assignee as the present invention.

By way of a summary account of one aspect of that invention, there was provided a thermocouple assembly having a core of insulating material within a tubular metallic housing surrounding a pair of spaced thermocouple conductors which projected beyond one end of the core in the housing to form a thermocouple junction. The opposite end of the housing was closed by terminal provisions for thermocouple connectors. A mounting apparatus was also disposed near that end to support the free junction end in a fluid stream which was subject to temperature measurement.

In a preferred embodiment of the invention, the major portion of the insulant was comprised of powdered magnesium oxide with the addition thereof of 20 percent by weight of a glass which had a softening point of 915° C. and a working point of 1200° C. The magnesium oxide and the glass were mixed in a finely divided form and compacted within the sheath to form an insulant about thermocouple leads. Thereafter, the entire assembly was subjected to a heat treatment which brought the insulating material up to a temperature of about 950° C. so that the glass portion of the mixture became slightly plastic. The temperature was not elevated enough, however, to cause the glass particles to flow. After cooling, the thermocouple assembly was found to possess

several distinct improved characteristics. The insulating material was mechanically strong but not brittle, and it was even possible to machine away portions of the outer sheath without the insulant crumbling or cracking under the strain.

5 Furthermore, thermal shock, so often encountered in the operation of such thermocouple assemblies, did not cause fracture of the rigid insulant. An additional important characteristic was that the insulant presented a nearly homogeneous barrier against the entrance of fuel or water vapor. Because the insulating material was not very porous and because the inherent toughness of the material resisted cracking under the most extreme conditions the thermocouple was likely to encounter, deterioration of the insulating value of the insulant due to the penetration of fuel or water vapor was greatly minimized. The thermocouple assembly had a considerably longer life, therefore, than most thermocouples previously designed to perform under the same conditions.

20 However, it was found subsequently that although the primary insulant material was itself impervious to passage of fuel or water vapors therethrough, some of these vapors did pass through the interfaces between the primary insulant and the sheath and between the primary insulant and the conductors.

25 The vapors passed into other areas at the end opposite to the thermocouple junction.

30 With this difficulty in mind, it is an object of this invention to provide a sheathed conductor which is highly resistant to fracture due to thermal and mechanical shock and relatively impervious to diffusion therethrough of water vapor for carbonizable fuels tending to decrease its effectiveness as an insulating agent by providing a seal which is impervious to the passage of fuel or water vapors therethrough and which bonds metallic oxide surfaces it contacts.

35 A further object of this invention is to provide a novel mineral insulating composition suitable for use in sheathed conductors for high temperature applications as a sealing material.

40 It is still another object of this invention to provide an improved method of producing such a sealing insulating composition.

### SUMMARY

45 By way of illustration, a sheathed conductor is hermetically sealed in accordance with this invention by depositing a quantity of sealing mixture in one end of a previously formed sheathed conductor including a primary insulating mixture.

50 The sealing mixture is composed of finely pulverized magnesium oxide and a finely pulverized glass having a thermal coefficient of expansion intermediate the coefficient of the sheath and the conductor and a working temperature which is less than the softening temperature of the primary insulant. The magnesium oxide constitutes 30-40 percent by weight of the sealing mixture. After cold pressing the sealing mixture against the sheath, conductors and primary insulant, the assembly is heated to the working point of the glass in the sealing mixture and then cooled so that the seal forms a bond with the sheath and with the conductors.

### BRIEF DESCRIPTION OF THE DRAWINGS

FIG. 1 is a partly pictorial cross-sectional view of a thermocouple assembly of the prior art to which this invention is adapted;

FIG. 2 is a block diagram illustrating a method of producing a seal for a sheath conductor according to the present invention;

FIG. 3 is a graph showing the heating steps necessary to produce the seal in accordance with this invention; and

FIG. 4 is a partly pictorial cross-sectional view of a thermocouple assembly constructed in accordance with the present invention.

## DESCRIPTION OF THE PREFERRED EMBODIMENTS

Although this invention can be applied to any sheathed conductor utilizing a primary insulating member, the invention can best be understood by referring to FIG. 1, which illustrates a thermocouple probe constructed in accordance with the method claimed in the referenced Clark et al. patent. The tubular thermocouple sheath or housing 10 is shown as extending through a wall 10' which is shown in phantom. To simplify the explanation, mounting means for such a probe are not shown as they are familiar to those skilled in the art. Tubular sheath 10 may be made of stainless steel or other suitable material, and a pair of thermocouple conductors 11 and 12 of dissimilar metals runs longitudinally therethrough, terminating in a protruding junction 13 at one end and in wires adapted to be connected to a utilization circuit 14.

Dissimilar conductors 11 and 12 may be of a type commonly employed in thermocouple pyrometry, one being a nickel-chromium alloy (90 percent nickel and 10 percent chromium) and the other being a nickel-aluminum alloy also containing small amounts of manganese and silicon (95 percent nickel, 2 percent aluminum, 2 percent manganese, and 1 percent silicon). Junction 13 may be rendered secure by welding. Insulation and positioning of conductors 11 and 12 is achieved by an insulating core 15.

As the composition of such insulants is well known, it suffices to state that in the Clark patent the insulant is a hard lime glass commercially available as Corning Type 1710 which has a softening point, at which it becomes slightly plastic, of about 915° C. and a working point, at which it is sufficiently liquid to be shaped or blown, of about 1200° C. Since glass is a super-cooled liquid, these temperatures, though known in the trade as "points," are in reality approximate temperature regions. The same glass, however, if exposed to some form of water, may acquire considerably elevated softening and working points, presumably as a result of chemical reaction with the carbon dioxide almost always present to some degree with the water. Because small particle sizes are employed, this chemical reaction, which ordinarily takes place in a very small scale, can be very significant.

The temperatures at which the particular primary insulant changes its physical properties are important and must be known if the present invention is to be practiced intelligently instead of by trial and error for, in the heat treatment operation to which the sheath conductor assembly is subjected, the temperatures should not exceed those which would soften components in the primary insulant. For example, in a thermocouple probe utilizing Corning Type 1710 glass in a homogeneous mixture with magnesium oxide, the temperature employed in obtaining the seal should not exceed 915° C.

FIG. 2 may be used as a ready reference guide to a comprehension of percent involved in the production of sealed sheath conductors according to the present invention. In an early percent-of-fabrication of the seal, magnesium oxide and glass are finely pulverized and mixed so that the magnesium oxide constitutes 30 percent-40 percent-weight of the final homogeneous seal mixture. When the filler of percent oxide is added, the seal is less susceptible to shock, apparently because the thermal gradient across any given increment of the glass is reduced. The particular glass which is chosen as a constituent in the seal mixture must have several properties. First, the thermal coefficient of expansion of the glass should be intermediate the thermal coefficients of expansion of the conductors and the sheath. Another characteristic of the glass is that it should, when mixed with the magnesium oxide, produce a material which is impervious to the entrance of fuel. Finally, the working point of the glass should be less than the softening point of any of the materials in the primary insulant.

For example, if the primary insulant is constituted by a mixture of 10 percent-30 percent of finely comminuted glass such as Corning Type 1710 and 70 percent-90 percent of magnesium oxide, a sealing mixture of 30 percent-40 percent by weight magnesium oxide with 70 percent-60 percent of a

lead-potash-soda combination such as Corning Glass Code 1990 formed in accordance with the method described hereinafter can be used. The thermal expansion of the sealing mixture approximately matches the thermocouple conductors and is less than the outer sheath expansion so the seal material is under compression with respect to the sheath after an initial firing process while very little or no stress is believed to be present at the conductors.

Although the remaining discussion of the production of a seal in accordance with this invention is directed to the particular constituent elements in the seal mixture, it will be obvious that the exercise of this invention can be varied and will be primarily dependent upon the materials from which the primary insulant, the sheath and the conductors are composed. When the Corning Glass Code 1990 and magnesium oxide mixture or other seal mixtures are used, the components should be finely pulverized and intimately mixed; for example, the glass-magnesium oxide mixture should be passed through a 325 mesh screen so as to exclude particles having a diameter greater than 1.7 mils. To form the seal, the mixture is then loaded into the thermocouple probe or other sheathed conductor and cold pressed at over 70,000 p.s.i. to reduce porosity and provide intimate contact between the glass and magnesium oxide particles. Thereafter, the mixture is subjected to a heat treatment according to the chart shown in FIG. 3.

Referring to FIG. 3, it will be seen that the time has been divided into six segments,  $T_1$ - $T_6$ . During the time  $T_1$ , the mixture is baked at a temperature which will drive off all moisture and purge air from the mixture. In the particular sealing mixture discussed above, the heating should be at about 475° C. for a period of at least four to five hours to assure that these two functions have been performed.

During the time segment  $T_2$ , the temperature is increased at a rate which is slow enough to induce some crystallization in the material but not so slow as to cause stratification of the material. Again referring to the particular sealing mixture, the temperature is linearly increased to about 750-760° C. during a 30-minute interval. Thereafter, the seal is stabilized at the upper temperature for a time segment  $T_3$ . The upper temperature limit is determined by the value above which a refractory like and weak composition results and the maximum time segment  $T_3$  is less than that which would cause stratification. For example, it is satisfactory to hold the glass-magnesium oxide mixture at 750-760° C. for five minutes.

During the time element  $T_4$ , the seal is cooled rapidly to prevent stratification without severely thermally shocking the seal. For example, the temperature could be dropped to about 550° C. in a period of approximately 20 minutes. Thereafter, slow cooling would be controlled so that the seal material and sheath and wires would cool uniformly to a point where the glass had become rigid, for example, to about 300° C. in about four hours. Thereafter, the seal is removed from the furnace.

The resulting structure is shown in FIG. 4 where like numerals designate like elements from FIG. 1. Again, the conductors 11 and 12 are in a primary insulant 15 which extends along a substantial portion of the length of the sheath 10. However, the seal 16 is shown as having been applied at one end thereof. It has been found that by following the above-described method, the seal 16 bonds to the metallic oxide of the sheath 10 and the conductors 11 and 12 so that fuel no longer can pass through the interfaces in the probe so the probe portions above the mounting plate 10' are maintained free of fuel vapors. It is believed that the magnesium oxide adds reinforcement to the composition to strengthen it and additionally promotes a degree of crystallization of the glass to thereby increase its resistance to cracking.

If magnesium oxide is used in a greater amount than the specified proportions, it becomes increasingly difficult to form the seal. This is believed to be caused by insufficient glass present in the mixture to bond to itself and the sheath to provide a continuous glass film and an impervious mass. If less than the specified proportions are used, the composition acts more like glass alone and is susceptible to cracking. There-

fore, other sealing mixtures should incorporate these parameters.

Thermocouple probes constructed in this invention have been evaluated for those thermal cycling and vibration conditions which are anticipated in jet engine applications. After subjecting thermocouple probes to such vibration and thermal cycling conditions, no significant leakage increases were measured with a mass spectrometer helium leak detector.

Therefore, in summary, this invention reveals a seal which can be adapted to any sheathed conductor when it is desired to prohibit the passage of carbonizable fuels or water vapor past a particular point. The seal is formed by utilizing a mixture of a finely pulverized glass which a working point which is less than a softening point for a primary insulating material with magnesium oxide, the magnesium oxide constituting 30 percent-40 percent by weight of the mixture. Thereafter, the mixture is subjected to cold pressing and a heat treatment to the working point of the glass material so that the seal bonds to adjacent metal surfaces.

While this invention has been described with particular reference to a particular thermocouple probe, the invention can be practiced with thermocouple probes formed by any number of materials without departing from the true spirit and scope of this invention. Therefore, it is desired that the appended claims cover all such variations and modifications which are within the true spirit and scope of this invention.

What is claimed as new and desired to be secured by Letters Patent of the United States is:

We claim:

1. A method for providing a hermetically sealed sheathed conductor comprising an outer sheath, an inner conductor, and a primary insulant extending over a substantial portion of the sheath length to space the conductor from the sheath including the steps of:

- a. filling a volume defined by an end surface of the primary insulant and the sheath with a mixture of finely divided magnesium oxide and a finely divided glass having a coefficient of thermal expansion intermediate the coefficients for the sheath and the conductor and having a working temperature which is less than the softening temperature of any constituent in the primary insulant, the composition consisting of 30 percent-40 percent by weight of the magnesium oxide;
- b. compacting the mixture to reduce porosity and provide intimate contact between the particles in the mixture;
- c. heating the sheathed conductor to remove moisture and purge air from the mixture;

5 d. elevating the temperature to the working temperature of the glass particles in the mixture at a rate which induces some crystallization without stratification for a time less than that which would induce stratification; and

e. cooling the sheathed conductor at a rate which prevents stratification without thermally shocking the seal.

2. A method for providing a sealed sheathed conductor comprising an outer sheath, an inner conductor and a primary insulant composed of a finely divided glass and a heat conducting material having a melting point above the softening point of the glass and selected from the class consisting of magnesium oxide, aluminum oxide, and beryllium oxide, with the glass being present in the mixture in the range of from 10 percent-30 percent by weight of the mixture, the primary insulant extending over a substantial portion of the sheath length to space the conductor from the sheath including the steps of:

- a. filling a volume defined by an end surface of the primary insulant and the sheath with a homogeneous mixture of magnesium oxide and a finely divided glass having a coefficient of thermal expansion intermediate the coefficients for the sheath and the conductors, the working temperature of the glass being less than the softening temperature for the finely divided glass in the primary insulant, the composition consisting of 30 percent-40 percent by weight of the magnesium oxide;
- b. compacting the mixture to reduce porosity in and to provide intimate contact between the particles;
- c. heating the sheathed conductor to remove moisture and purge air from the mixture;
- d. elevating the temperature of the sheathed conductor to the working temperature of the glass particles at a rate which induces some crystallization without stratification and thereafter maintaining the temperature at the working temperature for the glass for a time less than that which would otherwise induce stratification; and
- e. cooling the sheathed conductor at a rate which prevents stratification without thermally shocking the probe.

3. A method as recited in claim 2 wherein the finely divided glass is constituted by a soda-lead-potash glass.

4. A method as recited in claim 3 wherein the glass and magnesium are passed through a No. 325 mesh prior to mixing.

5. A method as recited in claim 4 wherein moisture is removed and air is purged from the mixture by maintaining the temperature at approximately 475° C. for more than four hours.